

## UNITED STATES PATENT OFFICE

CHESTER E. ADAMS, OF HAMMOND, INDIANA, ASSIGNOR TO STANDARD OIL COMPANY, OF WHITING, INDIANA, A CORPORATION OF INDIANA

## COLOR STABILIZATION OF LUBRICATING OILS

No Drawing.

Application filed June 8, 1928. Serial No. 284,016.

This invention relates to the color stabilization of lubricating oils and particularly hydrocarbon lubricating oils.

It is well known that during use, for example, in internal combustion engines, hydrocarbon oils rapidly deteriorate in color and appearance, and such deterioration is accompanied by more or less impairment of the oil in other respects.

10 I have found that by adding to such oils a relatively small proportion of suitable aliphatic amines, the deterioration of color is reduced to a remarkable extent.

15 In general, the amount of amine employed is preferably less than 1%. Even minute quantities of aliphatic amines, for example, of the order of 0.05% of the oil, give beneficial effects.

20 Primary, secondary and tertiary aliphatic amines are efficacious in preserving the color of the oil. However, it is preferred to employ the secondary and tertiary aliphatic amines on account of their lower volatility.

25 Substituted aliphatic amines, that is, amines in which one or more of the aliphatic groups contain hydroxyl and other substituted groups, may be employed. The hydroxy-alkylamines are especially preferred since they combine a high effectiveness with relatively low volatility. The presence of a large number of hydroxyl groups tends to render the amine insoluble in the oil and it is therefore preferred to employ aliphatic amines containing two hydroxy-alkyl groups

30 and one alkyl group.

35 Among the aliphatic amines which have been tested and found effective for the purpose may be mentioned butylamine, diethanolamine, ethyldiethanolamine, butyldiethanolamine, heptyldiethanolamine, cetyl-diethanolamine, tributylamine, tri-isoamylamine, di-isoamylamine and diethylcetylamine.

40 The efficacy of the present invention will be readily understood from the following specific example. A pale oil, derived from Mid-Continent crude, of color 35 on the true color scale, and having a viscosity of 200 seconds Saybolt (100° F.) was heated for 72 hours at about 250° F. At the end of that

50 period, its color was 200 +, that is, almost

black. Another example, to which 0.1% of butyldiethanolamine was added, was subjected to exactly the same treatment, and at the end of the test, it had a color of 42.

The remarkable improvement effected by the addition of aliphatic amines is unrelated to oxygen absorption since the amount of oxygen absorbed under the conditions specified above is not materially altered by the addition of the aliphatic amines.

I claim:

1. A hydrocarbon lubricating oil containing a small proportion of an aliphatic amine having an alkyl group containing not less than four carbon atoms.

2. A hydrocarbon lubricating oil containing a small proportion of an aliphatic amine having more than one aliphatic group each said aliphatic group having not less than four carbon atoms.

3. A hydrocarbon lubricating oil containing a small proportion of an aliphatic amine having at least one substituted-alkyl group.

4. A hydrocarbon lubricating oil containing a small proportion of an aliphatic amine having at least one hydroxy-alkyl group.

5. A hydrocarbon lubricating oil containing a small proportion of a tertiary aliphatic amine, each aliphatic group thereof having not less than 2 carbon atoms.

6. A hydrocarbon lubricating oil containing a small proportion of a tertiary aliphatic amine having at least one substituted-alkyl group.

7. A hydrocarbon lubricating oil containing a small proportion of a tertiary aliphatic amine having at least one hydroxy-alkyl group.

8. A hydrocarbon lubricating oil containing a small proportion of an aliphatic amine having two hydroxy-alkyl groups and a alkyl-group united to the nitrogen atom.

9. A hydrocarbon lubricating oil containing a small proportion of an aliphatic amine having two ethanol groups and an alkyl group united to the nitrogen atom.

10. A hydrocarbon lubricating oil containing a small proportion of butyldiethanol amine.

11. The method of color stabilizing hydro-

- bon lubricating oils which consists in adding thereto a small proportion of an aliphatic amine having an alkyl group containing at least four carbon atoms.
2. The method of color stabilizing hydrocarbon lubricating oils which consists in adding thereto a small proportion of an aliphatic amine having more than one aliphatic group containing at least four carbon atoms.
3. The method of color stabilizing hydrocarbon lubricating oils which consists in adding thereto a small proportion of an aliphatic amine containing at least one substituted-alkyl group.
4. The method of color stabilizing hydrocarbon lubricating oils which consists in adding thereto a small proportion of an aliphatic amine containing at least one hydroxy-alkyl group.
5. The method of color stabilizing hydrocarbon lubricating oils which consists in adding thereto a small proportion of a tertiary aliphatic amine, each aliphatic group thereof having at least 2 carbon atoms.
6. The method of color stabilizing hydrocarbon lubricating oils which consists in adding thereto a small proportion of a tertiary aliphatic amine containing at least one substituted-alkyl group.
7. The method of color stabilizing hydrocarbon lubricating oils which consists in adding thereto a small proportion of a tertiary aliphatic amine containing at least one hydroxy-alkyl group.
18. The method of color stabilizing hydrocarbon lubricating oils which consists in adding thereto a small proportion of an aliphatic amine having two hydroxy-alkyl groups and an alkyl-group united to the nitrogen atom.
19. The method of color stabilizing hydrocarbon lubricating oils which consists in adding thereto a small proportion of an aliphatic amine having two ethanol groups and an alkyl group united to the nitrogen atom.
20. The method of color stabilizing hydrocarbon lubricating oils which consists in adding thereto a small proportion of butyl-diethanolamine.
21. A lubricating oil comprising a hydrocarbon lubricant and a small proportion of an aliphatic amino compound having attached the amino nitrogen of the compound, substituting groups of the class consisting of aliphatic hydrocarbon radicals having more than 2 carbon atoms and the hydroxy-alkyl radicals.
22. A lubricating oil consisting of a hydrocarbon lubricant and a small proportion of an aliphatic amino compound wherein an aliphatic hydrocarbon radical having more than 2 carbon atoms and a hydroxy-alkyl radical are attached to the amino nitrogen atom, the remaining group attached thereto being of the class consisting of hydrogen and
- aliphatic hydrocarbon radicals having more than 2 carbon atoms.
23. The method of color stabilizing hydrocarbon lubricating oils which consists in adding thereto a small proportion of an aliphatic amino compound wherein an aliphatic hydrocarbon radical having more than 2 carbon atoms and a hydroxy-alkyl radical are attached to the amino nitrogen atom, the remaining group attached thereto being of the class including hydrogen and aliphatic hydrocarbon radicals. 70
24. The method of color stabilizing hydrocarbon lubricating oils which consists in adding thereto a small proportion of an aliphatic amino compound wherein an aliphatic hydrocarbon radical having more than 2 carbon atoms and a hydroxy-ethyl radical are attached to the amino nitrogen atom, the remaining group attached thereto being of the class consisting of hydrogen and aliphatic hydrocarbon radicals. 80
25. A hydrocarbon lubricating oil containing a small proportion of tributylamine.
26. The method of color stabilizing hydrocarbon lubricating oils which comprises adding thereto a small proportion of tributylamine. 90
27. The method of color stabilizing hydrocarbon lubricating oils which comprises adding thereto a small proportion of an aliphatic amine selected from the group consisting of butylamine, diethanolamine, ethyldiethanolamine, butyldiethanolamine, heptyldiethanolamine, cetyl diethanolamine, di-isoamylamine and diethylcetylamine. 95
28. The method of color stabilizing hydrocarbon lubricating oils which comprises adding thereto a small proportion of a tertiary aliphatic amine selected from the group consisting of tributylamine and tri-isoamylamine. 105
29. A hydrocarbon lubricating oil containing a small proportion of an aliphatic amine selected from the group consisting of butylamine, diethanolamine, ethyl diethanolamine, butyl diethanolamine, heptyl diethanolamine, cetyl diethanolamine, di-isoamylamine and diethylcetylamine. 110
30. A hydrocarbon lubricating oil containing a small proportion of a tertiary aliphatic amine selected from the group consisting of tributylamine and tri-isoamylamine. 115
31. A hydrocarbon lubricating oil containing a small proportion of a tertiary aliphatic amine, having alkyl groups containing at least four carbon atoms each. 120
32. A hydrocarbon lubricating oil containing a small proportion of butylamine. 125
33. The method of color stabilizing hydrocarbon lubricating oils which comprises adding thereto a small proportion of a butyl-amine.
34. The method of color stabilizing hydro- 130

carbon lubricating oils which comprises adding thereto a tertiary aliphatic amine having alkyl groups containing not less than four carbon atoms each.

35. A hydrocarbon lubricating oil containing a small proportion of a secondary aliphatic amine having alkyl groups containing not less than five carbon atoms.

36. A hydrocarbon mineral oil containing a small proportion of an aliphatic amine having an alkyl group containing not less than four carbon atoms.

In testimony whereof, I have hereunto set my hand this 27th day of April, A. D., 1928.

CHESTER E. ADAMS.

15

20

25

30

35

40

45

50

55

60

65